

Oct. 1, 1957

M. H. PARKS

2,808,247

MINING OF SULFUR BY LIQUEFACTION OF THE SULFUR

Filed Sept. 26, 1956



*Mercer H. Parks*  
ATTORNEY.

1

2,808,247

MINING OF SULFUR BY LIQUEFACTION  
OF THE SULFURMercer H. Parks, Houston, Tex., assignor to Humble  
Oil & Refining Company

Application September 26, 1956, Serial No. 612,328

6 Claims. (Cl. 262—3)

The present invention is directed to a method of mining sulfur. More particularly, the invention is concerned with the mining of sulfur from subsurface formations without causing subsidence of overlying formations. In its more specific aspects, the invention is directed to the mining of sulfur under controlled conditions whereby the pressure and volume of the ore body which contains the sulfur remains substantially under a constant pressure and at a substantially constant volume.

The present invention may be briefly described as a method for mining sulfur from a sub-surface earth formation containing a sulfur ore body by liquefaction of the sulfur. The invention specifically contemplates that all or major portions of the ore body will be heated as uniformly as possible to a temperature below the incipient melting point of the sulfur in the ore body. Thereafter, the temperature of the heated ore body is increased at least adjacent a well penetrating the ore body to a temperature sufficient to melt the sulfur in the region of or adjacent said well. Thereafter, the melted sulfur is produced through the well.

In accordance with the present invention the pressure and volume of the heated ore body is maintained substantially constant while producing sulfur from the ore body. This may be accomplished by injecting into the heated ore body a sufficient amount of water at an elevated temperature to liquefy or melt the sulfur in the heated ore body adjacent the production well and withdrawing from the heated ore body only a sufficient amount of fluid including melted sulfur and mine water sufficient to compensate for the amount of heated water injected into the ore body.

It is contemplated that the heated ore body will be substantially completely heated to a temperature below the incipient melting point of the sulfur in the ore body; for example, at a temperature below about 240° F. may be satisfactory. The temperature of 238° F. is exemplary of temperatures contemplated in the practice of the present invention. In heating the ore body to a temperature below the incipient melting point of the sulfur in the ore body, the heated water may be injected into the sulfur-bearing ore body incrementally. For example, the hottest water at a temperature of about 240° F. may be introduced into the upper part of the sulfur bearing formation or ore body and thereafter other increments of heated water at decreasing temperatures may be introduced below the upper layer of water introduced into the ore body such that the ore body is maintained at a temperature below the incipient melting point of the sulfur in the ore body.

In accordance with the present invention, it is contemplated that sulfur will normally be produced from the same wells used for water injection but may be produced from one well while heated mine water is introduced into another well. It is further contemplated that the first wells may be up formation from the second wells which are down formation from the first wells such that the sulfur progressively melted from the ore body and not

2

produced through water injection wells may be recovered by gravity drainage.

In the practice of the present invention a feature thereof is maintaining the ore body at a substantially constant pressure and volume to prevent subsidence of formations overlying the ore body. This may suitably be accomplished by filling the porous, barren cap which usually overlies a sulfur ore body with a suitable fluid which may be under pressure as desired. The suitable fluid may be mud, oil, water less saline than formation water, or it may be gas under pressure.

The present invention will be further illustrated by reference to the drawing in which the single figure illustrates a preferred mode. Referring now to the drawing, 15 numeral 11 designates a sulfur ore body which has a porous, barren cap rock 12 overlying same and above which are sedimentary deposits 13, 14, 15 and 16. The sulfur ore body may suitably be located beneath a body of water, such as, for example, in the Gulf of Mexico, or 20 suitably may be beneath the Coastal plains, such as in Texas or Louisiana. Drilled through the sedimentary formations 13 to 16 and to penetrate the porous, barren cap 12 is a borehole 17 in which is arranged a casing string 18 which is suitably cemented in place by cement 25 19. The casing 18 is penetrated to form perforations 20 into the porous, barren cap 12. Arranged within the casing string 18 is a water string 21 which extends into the borehole 22 of reduced diameter in the sulfur body 11. The annulus 23 between the water casing string 18 and the 30 water string 21 is suitably closed by a packer 24 of a type which will permit relative movement of water string 21 to casing string 18 without resetting or damaging the packer.

Arranged within the water string 21 is an inner pipe or 35 sulfur tubing string 25 and arranged within the inner pipe string 25 is a second inner pipe string 26 which suitably may be termed an air string. Water may be introduced down the annulus 27 between the string 25 and the water string 21 and sulfur may be produced upwardly through 40 the annulus 28 between the string 25 and the string 26 while air may be introduced downwardly through the string 26. The air string 26 is run in wells A only after the formation has been heated uniformly as noted before and sulfur production is to begin. It will be run in 45 wells B if air or gas lift is used to remove water from the formation as described.

The water string 21 is perforated by perforations 29 throughout its traverse of the sulfur ore body 11 and the sulfur string 25 is also provided with perforations 30 adequate to pass required volume of water above packer 31 between sulfur and water strings 25 and 21.

In providing a well of the nature described, it is desirable to seal the casing string 18 in the well bore 17 and to cement the water string 21 into the ore body 11 but not cement it to the casing string 18. In order to achieve this end, prior to running in the pipe strings 25 and 26, the lower portion of the water string 21 is sealed off by means of a drillable packer which may suitably be a cement plug, not shown, to isolate the uppermost of the 55 perforations 29 from the lowermost of the perforations and to squeeze cement through these upper perforations which may suitably be termed 29a and to cement the water string 21 by means of cement 32 into the sulfur ore body 11.

65 This may be accomplished without providing a drillable packer, not shown, in the water string 21 by first forming only the perforations 29a and then squeezing cement through the perforations 29a and removing excess fluid cement from the water string 21 followed by 70 forming the perforations 29 in the water string 21 after the cement 32 has been squeezed. It is contemplated that the perforations 20 and perforations 29 and 29a and

the perforations 30 may be formed in the several strings at the well head prior to placing the particular pipe string in the well or may be formed by gun perforating by lowering a perforator down through the respective strings prior to lowering the last string therethrough. In any event, it is contemplated that the several perforations may be provided.

The foregoing description refers to a first well A which may be drilled up formation in the sulfur ore body and a second well, which may be termed well B, may be subsequently drilled to penetrate the sulfur ore body down formation from the well A. The same procedure and the same elements are provided for well B and it is unnecessary to designate the several elements by different numerals. Accordingly, well A and well B have identical parts numbered identically. These wells are typical and it is contemplated that a number of each would be required in the proposed operation.

In practicing the present invention with wells A and wells B, as shown in the drawing, the first step to be employed if a porous, barren cap, such as 12, is above the sulfur ore body 11, is to fill the porous barren cap 12 with a suitable fluid which will prevent migration of the heated mine water up into the porous, barren cap. To this end, the suitable fluid, such as has been described, is forced down the annulus 23 and through the perforations 20 to fill the porous, barren cap with fluid and to prevent migration of mine water into the barren cap. As stated, this fluid may suitably be mud, oil, water, or gas. This fluid under pressure also serves to prevent subsidence of the overlying strata or formations 13 to 16 and to prevent collapse as the sulfur is mined from the ore body 11.

Heated mine water is then flowed down the annulus 27 at a temperature sufficient to heat the whole of the ore body 11 to a temperature below the incipient melting point of the sulfur in the ore body 11. In short, all or the major portion of ore body 11 is heated to a temperature below the melting point of sulfur, such that by raising the temperature of portions of the heated ore body adjacent the well, it is then possible to liquefy or melt the heated sulfur by raising the temperature of the ore body only slightly. Thus a relatively small quantity of heat will melt a relatively large quantity of sulfur in a very short time.

Once the heated ore body is heated to a temperature as has been described, the next step is the liquefaction of the sulfur adjacent or in the region of either wells A or B and to produce the sulfur from the annulus 28 using air or gas lift by introducing air or gas down through the inner pipe string 26.

As has been described briefly, the first step of the present invention is to fill the pores of the porous, barren cap rock with a fluid, such as has been indicated, to prevent convection of hot mine water into the formation 12. This introduction of a fluid, such as mud or water less saline than formation water, is usually through the wells A which are up structure from the wells B and is through the annulus 23 and perforations 20. The volume and temperature of this injected fluid are carefully controlled and a radioactive tracer element, such as tritium, having a half life of 12 years may be introduced therewith in order to follow the travel of the fluid. It is desirable to follow the travel of the fluid in the porous, barren cap such that the fluid travels toward all of the surrounding wells of which well B may be representative.

In order to maintain this travel, it may be desirable to bleed fluid from well B, for example through the annulus 28, to cause a differential pressure between wells A and B to induce movement of fluid from well A to well B. Of course, it is desirable simultaneously to maintain reservoir pressure by a careful control of the injection fluid and control of the withdrawn fluid. Travel, as correlated to injection and withdrawal, can suitably be determined by testing the withdrawn water or fluid

from well B for the radioactive tracer element and by determining its temperature.

This operation is continued until the porous, barren cap rock is satisfactorily filled or until it has been filled sufficiently to accomplish the end of preventing migration of heated mine water.

Thereafter the injection of hot water begins at wells A. The sulfur tubing string 25 may be set so that the packer 31 in wells A exposes only a few feet of perforations 29 near the top of the sulfur ore body 11. This water may be first injected at 315° F. or higher but a careful control thereof is desirable such that little, if any, of the sulfur in the body 11 is melted. As the temperature of the ore body 11 rises to approximately 238°

15 or 240° F. or a suitable point below the sulfur melting point in the upper part of the sulfur ore body 11, the packer 31 is lowered and the water temperature may be decreased slightly with the volume of the water correspondingly increased to deposit a layer of water 20 below the layer of water at 238° F.; for example, the second layer of water may be below 238° F. followed by a third layer of water and other layers of water at progressively lower temperatures as may be desired. As the ore body 11 becomes progressively heated, some of 25 the wells B may be made injection wells for injection of hot water to aid in the heating of the ore body 11 in the region of the wells B. As an alternate to heating by the creation of layers of progressively cooler water as the lower parts of the formation are filled, it is contemplated 30 that a simplification might accomplish the purpose of preheating simply by injecting water between 240° F. and 315° F. through the lower perforations of water string 21, such as it would be injected for regular Frasch mining, except that care would be exercised to prevent 35 the melting of appreciable amounts of sulfur.

When hot water injection is started at wells A, bleeding of water is started at wells B through the annulus 27 or water string 21, alone, at a rate not only to maintain the pressure within the reservoir 11 but to maintain its 40 volume substantially constant taking into consideration the expansion characteristics of all reservoir material and the physical changes in the rock as it becomes depleted of its sulfur. Thus, a sufficient amount of hot water is injected to compensate for the amounts of bleed water 45 and sulfur, if any, withdrawn.

It is possible also to be injecting fluid into the porous, barren cap 12 simultaneously with the heating of the sulfur ore body 11 provided, of course, that the amount of fluid injected into barren cap 12 and its course have 50 been determined such that convection does not cause the hot water injected to heat the ore body 11 to migrate into the cap 12.

It is recognized that the sulfur in the ore body 11 supplies a considerable portion of the strength of the 55 cap rock 12 to resist the crushing of the overlying strata or formations 12 to 16. In the mining of sulfur, subsidence is a problem. In accordance with the present invention the sulfur is prevented from melting until it is desired to produce the sulfur such that it may be 60 produced in a volume sufficient such that the volume as well as the pressure in the ore body 11 may be maintained substantially constant in order to prevent overloading of the cap rock or barren cap 12 at any stage of the heating or of the sulfur melting. While the volume of the water and sulfur removed from wells A or B may be followed to determine the maintenance of the volume in the formation, another method of following the maintenance of pressure and volume of the formations is by hanging the water string 21 in the top part of the sulfur ore body 11 by means of the squeeze cement 32. The weight of the pipe in the string 21 may be set down on this cement 32 and the remainder of the weight may be carried by a weight indicator device at the top of the 65 hole which, by registering an increased load, will indicate incipient failure through melting of the sulfur

from around the cement plug with slippage of the casing 21 through the packer 24. Alternately, the movement of the casing 21 may be noted at the surface through levelling same with respect to a fixed elevation. Differential movement of strings 18 and 21 may also be a control for the maintenance of the pressure and volume of the sulfur ore body 11 and a porous, barren cap 12.

After the sulfur ore body 11 has been substantially completely heated to a temperature about or below 240° F., the air or gas lines 26 may be run into the well and a temperature of the injected water increased to about 315° F. with the result that the sulfur in the ore body 11, which is below incipient melting point, may be supplied with the necessary heat input for fusion and melting to take place with the employment of a relatively small amount of hot water per ton of sulfur produced. In short, the wells A and B may then be produced under control by controlling the volume of fluids in the reservoir constant by controlling the bleed water with respect to the water injected and the sulfur removed, other conditions, such as temperatures and pressures also being controlled. Thus, in the present invention it is essential that the reservoir configuration be maintained substantially unchanged through maintenance of equilibrium within it and thus prevent subsidence with the attendant slippage of formations which destroys wells and interrupts production by subsurface and surface dislocations.

It is contemplated in the practice of the present invention that if the sulfur becomes depleted from the highest point in a formation or strata of a sulfur ore body that that portion of the porous, barren cap and its overlying strata may be caused to collapse by deliberately bleeding through a well B to reduce volume and thereby force the fluids within the depleted portion of the sulfur ore bodies out and down formation to heat that portion of the formation such as is adjacent to a well B.

In the practice of the present invention where the porous, barren cap rock is filled with a substance to prevent ingress of hot water while the ore body is heated to a temperature below the incipient melting point of the sulfur in the ore body, it may be desirable to employ water of lesser density than that in the formation. For example, sea water having a density of slightly over 1.0 might be employed to displace cap rock water of a density of as much as 1.1 to 1.2, reducing the difference in cap rock water and heated sea water having a density of from about 0.95 to 0.91 used to heat the sulfur ore body. In other words, by selecting the density of the water employed to fill the porous, barren cap rock, the tendency of the water to migrate into the porous, barren cap rock may be controlled.

The present invention is of considerable importance and utility in that the number of wells employed and the attendant operating equipment is substantially reduced. The sulfur is substantially completely mined from the ore body with a minimum amount of water and heat input and subsidence of overlying strata or formations is substantially completely eliminated.

The nature and objects of the present invention having been completely described and illustrated, what I wish to claim as new and useful and to secure by Letters Patent is:

1. A method for mining sulfur from a subsurface earth formation containing a sulfur ore body by liquefaction of the sulfur which comprises introducing into said ore body a sufficient amount of heated water at a sufficient temperature to heat said ore body and to raise the temperature of the ore body to a temperature below the incipient melting point of sulfur in said ore body, then raising further the temperature of the heated ore body at least adjacent a well penetrating said ore body a sufficient amount to melt the sulfur in said heated ore body adjacent said well, and then producing melted sulfur and water through said well, the pressure and volume of said heated ore body being maintained substantially constant by controlled injection of heated water into the heated ore body under pressure and at a rate sufficient to compensate for the amount of melted sulfur and water produced from the heated ore body, the heated water injected into the heated ore body by controlled injection being at a temperature sufficient to raise the temperature of the heated ore body to melt the sulfur.
2. A method for mining sulfur from a subsurface earth formation containing a sulfur ore body by liquefaction of the sulfur which comprises heating said sulfur ore body to a temperature below the incipient melting point of the sulfur in said ore body, increasing the temperature of the heated ore body adjacent a well penetrating said ore body to a temperature sufficient to melt the sulfur in said ore body adjacent said well, and then producing melted sulfur and water through said well, the pressure and volume of said heated ore body being maintained substantially constant by controlled injection of heated water into the heated ore body under pressure and at a rate sufficient to compensate for the amount of melted sulfur and water produced from the heated ore body, the heated water injected into the heated ore body by controlled injection being at a temperature sufficient to raise the temperature of the heated ore body to melt the sulfur.
3. A method in accordance with claim 2 in which the ore body is heated to a temperature below approximately 240° F.
4. A method in accordance with claim 2 in which the ore body is heated to a temperature below the incipient melting point of the sulfur in the ore body by injection of heated water through a first well penetrating said ore body and melted sulfur is produced through a second well penetrating said ore body down formation from the first well.
5. A method in accordance with claim 2 in which the sulfur ore body is heated to a temperature below the incipient melting point of sulfur by injecting in sequence increments of heated water at progressively decreasing temperatures to maintain the temperature of the ore body below the melting point of sulfur.
6. A method in accordance with claim 5 in which the increments of heated water of decreased temperature are injected into said ore body below increments of heated water at a higher temperature.